

# UNITED STATES PATENT OFFICE.

EARL BLOUGH, OF PARNASUS, PENNSYLVANIA, ASSIGNOR TO ALUMINUM COMPANY OF AMERICA, OF PITTSBURGH, PENNSYLVANIA, A CORPORATION OF PENNSYLVANIA.

## HEAT TREATMENT OF ALUMINUM ALLOYS.

1,394,534.

Specification of Letters Patent.

Patented Oct. 25, 1921.

No Drawing. Application filed November 30, 1917, Serial No. 204,540. Renewed December 28, 1920. Serial No. 433,691.

To all whom it may concern:

Be it known that I, EARL BLOUGH, a citizen of the United States, residing at Parnasus, in the county of Allegheny and State of Pennsylvania, have invented certain new and useful Improvements in Heat Treatment of Aluminum Alloys, of which the following is a full, clear, and exact description.

This invention relates to the heat treatment of aluminum alloys, and the chief object of the invention is to provide a simple and easily worked method of treatment for the purpose of improving the important physical properties of hardness and tensile strength, especially the latter.

As in the treatment of steel, certain prior processes or methods involve heating the metal and then cooling or quenching it. The present invention is based on the discovery that the heat-treatment should be effected in stages, the first at a rather elevated temperature and the last at a somewhat lower degree.

In applying my process in the preferred manner, the metal is first heated to a temperature of about 500° C. or higher, say 575° or more, but in general not above 600°. In many cases 520° is satisfactory. The temperature may be considerably lower, for example around 400°, but a higher degree is better. In general, the duration of this heating stage should be long enough for the metal to reach a state of equilibrium, that is to say, a state in which any internal stresses and strains have been relieved and in which there have taken place any thermal reactions and changes that normally occur at such temperature, as for example change in the crystalline structure of the alloy.

The actual time required for this effect is of course variable with the nature of the alloy, but ordinarily a period of from two to three hours heating, after the metal has been brought up to the temperature, has been found sufficient. If such a period does not

give the desired results in any specific instance longer periods may be tried. The heating is now continued (without intermediate rolling, stamping, drawing or other working) at a lower temperature, which may be between about 100° and about 200°. Good results are secured at 100°, and this temperature is advantageous because of the convenience with which it can be obtained and maintained by means of boiling water. With

temperatures much above 200°, say 250°, it 55 has been observed that the elongation is apt to be impaired and the improvement in tensile strength diminished. A time of two hours for the second heating is ample for most purposes, but it may be prolonged beyond that. I have not, however, observed any material advantage in continuing the second heating longer than about twenty-four hours. Instead of continuing the second heating stage it may be maintained 60 merely long enough for the lower temperature to become uniform throughout the metal, after which the temperature can be raised, say to between 150° and 200°, about, and kept there until the results desired are 65 attained.

The metal can now be cooled, quickly or slowly, whereupon it will be found that its tensile strength has been very remarkably increased. Nor is it necessary to store the 75 metal, or allow it to rest, for a time after cooling, before it is used. On the contrary, the metal can at once be put to any use for which it is suitable. In fact, with a final heating stage or step lasting no more than 80 twenty-four hours the tensile strength has been found to be superior to that resulting from four days storing after cooling following a single heating.

My process is applicable to a great variety 85 of aluminum-copper alloys, and to aluminum-copper alloys containing also one or more of other metals, for example, zinc, magnesium, iron, calcium, and silicon. It is particularly effective with alloys in which the 90 copper content does not exceed about ten per cent.

The temperatures referred to in the foregoing description and in the appended claims are all measured on the centigrade 95 scale.

I claim:—

1. In a method of heat-treating aluminum alloy of the kind described to improve certain of its physical properties, especially 100 tensile strength, the steps comprising subjecting the said alloy to heat at a temperature above about 400° C., and, without working the alloy, subjecting it for a period of time to heat at a lower temperature. 105

2. In a method of heat-treating aluminum alloy of the kind described, to improve certain of its physical properties, especially

tensile strength, the steps comprising subjecting the alloy to heat at a temperature of above about 400° C., and, without working the alloy, subjecting it for a period of time 5 to heat at a temperature not less than about 100° C.

3. In a method of heat-treating aluminum alloy of the kind described, to improve certain of its physical properties, especially tensile strength, the steps comprising subjecting the said alloy to heat at a temperature of not less than about 500° C., and, without working the alloy, subjecting it to further heating for a period of time at a lower temperature. 10

4. In a method of heat-treating aluminum alloy of the kind described, to improve certain of its physical properties, especially tensile strength, the steps comprising subjecting the alloy to heat at a temperature of not less than about 500° C., and, without working the alloy, subjecting it to further heating for a period of time at a temperature of not less than about 100° C. 20

5. In a method of heat-treating aluminum alloy of the kind described, to improve certain of its physical properties, especially tensile strength, the steps comprising subjecting the alloy to heat at a temperature 30 above about 400° C., and, without working the alloy, subjecting it to further heating at a lower temperature for a period of not less than about two hours. 25

6. In a method of heat-treating aluminum alloy of the kind described, to improve certain of its physical properties, especially tensile strength, the steps comprising subjecting the alloy to heat at a temperature above about 400° C., and, without working 40 the alloy, subjecting it to further heating at a temperature of not less than about 100° C., for a period of not less than about two hours.

7. In a method of heat-treating aluminum alloy of the kind described, to improve certain of its physical properties, especially tensile strength, the steps comprising subjecting the alloy to heat at a temperature of not less than about 500° C., and, without 50 working the alloy, subjecting it to further heating at a lower temperature for a period of not less than about two hours.

8. In a method of heat-treating aluminum alloy of the kind described, to improve certain of its physical properties, especially tensile strength, the steps comprising subjecting the alloy to heat at a temperature not less than about 500° C., and, without working the alloy, subjecting it to further heating at a temperature of not less than about 100° C., for a period of not less than about two hours. 60

9. In a method of heat-treating aluminum alloy of the kind described, to improve certain of its physical properties, especially 65

tensile strength, the steps comprising subjecting the alloy to heat at a temperature above about 400° C., then, without working the alloy, subjecting it to heat at a temperature above about 100° C., and then, without working the alloy, subjecting it for a period of time to heat at a higher temperature than that used in said second step but below 300° C. 70

10. In a method of heat-treating aluminum alloy of the kind described, to improve certain of its physical properties, especially tensile strength, the steps comprising subjecting the alloy to heat at a temperature above about 500° C., then, without working 75 the alloy, subject it to heat at a temperature above about 100° C., then without working the alloy subjecting it for a period of time to heat at a higher temperature than that used in said second step, but below 300° C. 80

11. In a method of heat-treating aluminum alloy of the kind described, to improve certain of its physical properties, especially tensile strength, the steps comprising subjecting the alloy to heat at an elevated temperature, then, without working the alloy, lowering its temperature materially; then, without working the alloy, raising its temperature and maintaining it for a period of time at a temperature materially higher 95 than that to which the temperature had been so reduced, but lower than that at which the alloy was subjected in such first step. 90

12. In a method of heat-treating aluminum alloy of the kind described, to improve certain of its physical properties, especially tensile strength, the steps comprising subjecting the alloy to heat at an elevated temperature, then, without working the alloy, lowering its temperature materially; then, 100 without working the alloy, raising its temperature and maintaining it for not less than two hours at a temperature materially higher 105 than that to which the temperature had been lowered, but lower than that at which the alloy was treated in the first step. 110

13. In a method of heat-treating aluminum alloy of the kind described, to improve certain of its physical properties, especially tensile strength, subjecting the alloy to heat 115 in a plurality of stages without intermediate working, at least two of the stages each lasting for a material period of time; the first at a temperature exceeding 400° C., and another at a temperature more than 200° C. 120 lower than the first.

14. In a method of heat-treating aluminum alloy of the kind described, to improve certain of its physical properties, especially tensile strength, subjecting the alloy to 125 heat in a plurality of stages without intermediate working, at least two of the stages each lasting for a sufficient length of time to establish the internal structure of the alloy in an approximately stable state at 130

that temperature, the temperature in the first of said stages exceeding 400° C., and the temperature in a subsequent one of said stages being more than 200° C. lower than

5 that in the first stage.

15. In a method of heat-treating aluminum alloy of the kind described, to improve certain of its physical properties, especially tensile strength, subjecting the alloy to heat

10 in a plurality of stages without intermediate working, at least two of the stages each lasting for a sufficient length of time to establish the internal structure of the alloy in an approximately stable state at that temperature, the temperature in the first stage exceeding 400° C., and the temperature in another of said stages being between 100° C. and 250° C., approximately.

15. In a method of heat-treating aluminum alloy of the kind described, to improve certain of its physical properties, especially tensile strength, subjecting the alloy to heat at an elevated temperature until the internal stresses existing have been relieved and the thermal reactions and changes that normally occur at such a temperature have taken place, and thereafter subjecting the alloy, without intermediate working, to heat at a lower temperature for a material period of

20 time.

17. In a method of heat-treating aluminum alloy of the kind described, to improve certain of its physical properties, especially tensile strength, subjecting the alloy to heat at an elevated temperature until the internal stresses existing have been relieved and the thermal reactions and changes that normally occur at such a temperature have taken place, and thereafter subjecting the alloy, without intermediate working, to heat at a lower temperature above about 100° C. for a material period of time.

18. In a method of heat-treating aluminum alloy of the kind described, to improve certain of its physical properties, especially tensile strength, subjecting the alloy to heat at an elevated temperature until the internal stresses existing have been relieved and the thermal reactions and changes that normally occur at such a temperature have taken place, and thereafter subjecting the alloy, without intermediate working, to heat at a lower temperature for not less than about two hours.

19. In a method of heat-treating aluminum alloy of the kind described, to improve certain of its physical properties, especially tensile strength, subjecting the alloy to heat at an elevated temperature until the internal stresses existing have been relieved and the thermal reactions and changes that normally occur at such a temperature have taken place, and thereafter subjecting the alloy, without intermediate working, to heat at a

lower temperature between about 100° C. and 300° C., for not less than about two hours.

20. In a method of heat-treating aluminum alloy of the kind described, to improve certain of its physical properties, especially tensile strength, subjecting the alloy to heat at a temperature of above 400° C., and, without working the alloy, quenching it in boiling water; then, without intermediate working, heating it in boiling water for a material period of time.

21. In a method of heat-treating aluminum alloy of the kind described, to improve certain of its physical properties, especially tensile strength, subjecting the alloy to heat at a temperature of over 400° C., and, without working the alloy, quenching it in boiling water; then, without intermediate working, heating it in boiling water for not less than about two hours.

22. In a method of heat-treating aluminum alloy of the kind described, to improve certain of its physical properties, especially tensile strength, subjecting the alloy to heat at a temperature of over 500° C., and, without working the alloy, quenching it in boiling water; then, without intermediate working, heating it in boiling water for a material period of time.

23. In a method of heat-treating aluminum alloy of the kind described, to improve certain of its physical properties, especially tensile strength, subjecting the alloy to heat at a temperature of over 500° C., and, without working the alloy, quenching it in boiling water; then, without intermediate working, heating it in boiling water for not less than about two hours.

24. In a method of heat-treating aluminum alloy of the kind described, to improve certain of its physical properties, especially tensile strength, subjecting the alloy to heat at a temperature of over 400° C., and, without working the alloy, quenching it in boiling water; then, without intermediate working, subjecting it to a further heating at a temperature between about 100° C. and 300° C., for a material period of time.

25. In a method of heat-treating aluminum alloy of the kind described, to improve certain of its physical properties, especially tensile strength, subjecting the alloy to heat at a temperature of over 500° C., and, without working the alloy, quenching it in boiling water; then, without intermediate working, subjecting it to a further heating at a temperature above about 100° C. for not less than about two hours.

In testimony whereof I hereunto affix my signature.

EARL BLOUGH.